

July 27, 1943.

H. HABART ET AL

2,325,314

METHOD OF MAKING HOLLOW ARTICLES

Filed Aug. 2, 1940



INVENTORS:

HERBERT HABAET and HARRY W. HUDSON,  
BY: John E. Jackson,  
THEIR ATTORNEY.

## UNITED STATES PATENT OFFICE

2,325,314

## METHOD OF MAKING HOLLOW ARTICLES

Herbert Habart and Harry W. Hudson, Ellwood City, Pa., assignors to National Tube Company, a corporation of New Jersey

Application August 2, 1940, Serial No. 350,154

## 1. Claim. (Cl. 29—156)

This invention is concerned with the piercing of solid stainless steel billets in a seamless tube piercing mill when the steel contains about 25% chromium and about 20% nickel.

In the manufacture of seamless tubes it is considered preferable to pierce solid billets rather than billets that have been drilled. Prior to the present invention it has been commercially impossible to pierce solid stainless steel billets of the above chromium and nickel content because the load placed on the mill during the piercing was more than a mill of standard design could carry.

The accompanying drawing schematically illustrates the present invention, the drawing being legend so that it is unnecessary to make specific reference to the various parts by numbers.

According to the present invention, while the stainless steel is molten its manganese content is adjusted to from more than 2% to not more than 4% while keeping the other constituents of the steel within the commercial range usual to its 25% chromium and 20% nickel content, the steel being rolled to solid billets when it solidifies and these billets being pierced in a seamless tube piercing mill. The pierced billets subsequently may be processed to finished tubes by conventional methods, it being possible to produce tubes with relatively thin walls. The characterizing feature is the adjustment of the manganese content, it having been found that when the manganese exceeds 2% the load on the piercing mill is materially reduced so that the mill can be commercially operated with safety and without incorporating any features uncommon to piercing mills satisfactory for use in piercing stainless steels of lower chromium and nickel content.

It is to be understood that the stainless steel with which the present invention is concerned is commercially known as 25-20 stainless and its usual commercial analysis for seamless tubes is:

|            | Percent     | 45 |
|------------|-------------|----|
| Chromium   | 24 to 26    |    |
| Nickel     | 19 to 21    |    |
| Carbon     | maximum .20 |    |
| Phosphorus | do .03      |    |
| Sulphur    | do .03      |    |
| Silicon    | do .75      | 50 |
| Iron       | Balance     |    |

In the above analysis the manganese content is not given since it is increased from usual to from more than 2% to less than 4% in the case of the present invention. This increase in the manganese content does not affect harmfully the stainless or other characteristics of the steel. The main effect of the manganese appears to be the reduction in the load on a piercing mill from a point where the load is too high to be safely carried by a standard mill to one where it is within safe limits. As a matter of fact, the pierceability of 25-20 stainless with its manganese content adjusted as described, is better than that of 18-8 stainless.

15 It is also to be understood that a seamless tube piercing mill as contemplated herein consists of diagonal rolls which grip the billet and work it over a piercing point positioned in the pass of the rolls by a mandrel bar. As previously mentioned, 20 the present invention permits 25-20 stainless in the form of solid billets to be pierced by such a mill without loading the mill beyond its working limit as is the case when an attempt is made to 25 pierce solid billets of 25-20 stainless of the usual analysis.

## We claim:

A method of making stainless steel hollow articles in a seamless tube piercing mill when said steel contains about 25% chromium and about 20% nickel, said method including preparing said steel for piercing by adding manganese while said steel is molten to give said steel a manganese content of from more than 2% to not more than 4% while keeping the other constituents of said steel within usual commercial ranges, rolling said prepared steel to solid billets when it solidifies and subsequently piercing said prepared solid billets in a seamless tube piercing mill, said manganese content causing a material reduction 40 in the load on said mill during said piercing.

HERBERT HABART.  
HARRY W. HUDSON.